

T. J. Mayall,  
Knife Sharpener.

No. 26,277.

Patented Nov. 29, 1859.



Witnesses:  
John Garrett  
Albert W. Brown

Testimony:  
T. J. Mayall

# UNITED STATES PATENT OFFICE.

THOMAS J. MAYALL, OF ROXBURY, MASSACHUSETTS.

## STEEL.

Specification of Letters Patent No. 26,277, dated November 29, 1859.

*To all whom it may concern:*

Be it known that I, THOMAS J. MAYALL, of Roxbury, in the county of Norfolk and State of Massachusetts, have invented certain new and useful Improvements in Steels or Implements Used for Sharpening Table-Knives, &c., and that the following description, taken in connection with the accompanying drawings hereinafter referred to, forms a full and exact specification of the same, wherein I have set forth the nature and principles of my said improvements by which my invention may be distinguished from all others of a similar class, together with such parts as I claim and desire to have secured to me by Letters Patent.

The figures of the accompanying plate of drawings represent my improvements.

Figure 1 is a plan or top view of my improved "steel." Fig. 2 is a central, longitudinal vertical section of the same. Figs. 3 and 4 are sectional views showing the molds.

The object of my invention is to form a "steel" for sharpening table knives, &c., which shall be cheaper and more durable than those heretofore manufactured. I accomplish these results by making the "steel" of india rubber or gutta-percha, combined with emery, sand or other gritty materials and sulfur compounded in any desired proportions. I make a composition of about the following proportions, viz: 15 lbs. of emery, sand or other gritty materials, 1 lb. of rubber or gutta-percha and 5 oz. of sulfur. These ingredients are perfectly combined and mixed together and the composition thus formed is then placed in metallic molds *a*—*b*—*b*, subjected to pressure and heated from fifteen minutes to four hours at a temperature of from 260° to 300° Fahrenheit, much less time being required when a high pressure is used than when a low pressure

only is obtained. This composition thus becomes hard and durable. The handle *c* can be formed in the molds, of hard-gum compound, at the same time with the above named composition, or of wood, metal, or other suitable material and both the inner body and handle of the "steel" may be of other substances than the composition above named, the sharpening composition being formed in sufficient thickness upon the said inner body in the molds.

The composition above stated and the degrees of heat to be employed admit of many variations and therefore I do not limit myself to the proportions named or to the degree of heat to be employed.

In order to give sufficient strength to the "steel," I use a piece of metal in the form of a tapering rod or otherwise, for the center. The emery composition is placed upon the outside of this metallic center before it is heated. I have found it best in practice to cover this metallic center with a thin coat of liquid rubber cement which causes the emery coating to adhere more perfectly to the metal. Wood or other stiff substances can be used in place of the metal, but they are not desirable substitutes.

Having thus described my improvements I shall state my claim as follows.

What I claim as my invention and desire to have secured to me by Letters Patent, is—

As a new article of manufacture, a "steel" or implement for sharpening table knives &c., formed of india-rubber or gutta-percha with which emery, sand, or other suitable gritty substances are incorporated, substantially as set forth.

THOS. J. MAYALL.

Witnesses:

JOSEPH GAVETT,  
ALBERT W. BROWN.